

M. R. TREMBOUR.  
METHOD OF OPERATING AN ELECTRIC FURNACE.  
APPLICATION FILED MAR. 24, 1916.

1,339,428.

Patented May 11, 1920.



Fig. 1



Fig. 2



Fig. 3



Fig. 4

Inventor

by Max R. Trembour,

Frederick W. Cameron, Atty.

# UNITED STATES PATENT OFFICE.

MAX R. TREMBOUR, OF WATERVLIET, NEW YORK, ASSIGNOR, BY MESNE ASSIGNMENTS, TO LUDLUM ELECTRIC FURNACE CORPORATION.

## METHOD OF OPERATING AN ELECTRIC FURNACE.

1,239,428.

Specification of Letters Patent. Patented May 11, 1920.

Application filed March 24, 1916. Serial No. 86,419.

To all whom it may concern:

Be it known that I, MAX R. TREMBOUR, a subject of the German Emperor, residing at the city of Watervliet, in the county of Albany and State of New York, have invented 5 certain new and useful Improvements in Methods of Operating an Electric Furnace, of which the following is a specification.

My invention is a new method of melting 10 and refining metals and alloys by means of electrical heating, and is especially adapted for use in the electric furnace described in my copending application on electric furnaces.

It has heretofore been believed by metallurgists that contact of a carbonaceous electrode with a molten charge of metal, such as iron or steel, would result in an excessive absorption of carbon by the metal from the 15 electrode. For this reason great care has been exercised and various processes have been developed to maintain such electrodes out of contact with the metal-charge. When in some types of furnaces electrical contact 20 has been made to the molten metal an artificially cooled metal-electrode has been resorted to, or the use of electrically conducting refractory furnace-linings has been recommended.

I have found, however, that under certain 25 conditions this absorption of carbon by the metal is so slow, particularly when a graphitic electrode is used, that during ordinary furnace operation the amount absorbed is quite negligible and is in fact less than required in any event for the great majority 30 of electric-furnace products. These conditions can be obtained by means of an adjustable electrode introduced into the furnace from above the level of the charge and in adjusting this electrode, when the current 35 is flowing, in such a way that it contacts with the metal so as to convey the current without appreciable heating effect at the 40 contact points and withdrawing this electrode from contact with the metal when no current is flowing, unless it is intended to carbonize the metal by means of the electrode-carbon.

In accordance with my present invention, 45 I have taken advantage of this discovery to provide an improved process of refining molten metals, whereby electrical heat is applied to the metal and to the refining slag 50 by means of adjustable carbonaceous elec-

trodes, at least one of which contacts with the metal without appreciable heating effect, while at least one electrode is spaced away from the metal without contacting and at such a distance as to produce the proper 60 heating effect, forcing the current to pass through the refining slag, which, according to chemical composition and physical properties, will offer more or less electrical resistance.

I have also provided an improved process for the melting and refining of a metal charge, whereby the same electrical equipment is used for both phases of the process, in such a way that during the melting period, 70 when the furnace and its contents are still relatively cold, all the electrodes are adjusted in such a way as to generate heat, while during the refining process at least one electrode is adjusted to contact with the 75 metal, thus eliminating the heating effect of the same and transferring it to the other electrode or electrodes, which are kept spaced away from the metal without contacting. The electric current employed in this process must be of a tension sufficient to 80 bridge air-gaps and poor contacts by an arc and to force its way through semi-conductive material such as slag, for which purpose a voltage of around 100 volts between the 85 phases has been found very satisfactory for a basic furnace, while an acid furnace requires a still higher voltage.

In the preferred embodiment of my invention the process is carried out in an oblong 90 furnace chamber with a charging door, 3, at each end of the longer axis; an electrode, 4 and 6, near each door where the dissipation of heat is greatest; and an electrode, 5, near the center of the furnace. This furnace is described in the copending application and shown in the accompanying drawing, in which:

Fig. 1 is a plan.

Fig. 2 is a section along the lines, *a—a*, on Fig. 1.

Fig. 3 is a section along the lines, *b—b*, on Fig. 1.

Fig. 4 is a side elevation.

Similar letters refer to similar parts throughout the several views.

Cold metal scrap may be heated and melted in this furnace in any convenient way, for instance, by striking an arc to the metal from each electrode, thus distributing

65

70

75

80

110

the heat throughout the chamber, which is desirable when the furnace is cold and the doors are kept closed.

When a fluid metal bath, 7, has been obtained and the same has been covered with the refining slag, 8, the middle electrode, 5, is lowered through the slag to contact with the metal. This at once increases the heating effect at the lower ends of the outside electrodes, 4 and 6, at the same time lowering the temperature in the center of the furnace. In other words, the heat is generated and applied to the metal and slag near the doors, where at the time of refining it is mostly needed, due to the fact that the doors must be opened repeatedly for observing and manipulating the slag, for sampling and for making additions. Applying the heat where it is needed, not only saves electric power, but also prevents over-heating of the refractory furnace lining near the central region of the furnace and thereby lengthens the life of this lining.

When melting down a cold charge, the metal directly under and around the electrodes melts away quickly and collects at the bottom of the furnace, forming there a pool of melted metal, or a bath, while the rest of the charge is still in process of melting. If this pool is covered with a proper slag, refining will begin right there. It is therefore not necessary to wait with the refining until the whole charge is melted, but it may be started as soon as a bath is formed, and an electrode may be contacted with the metal while the melting process is still carried on.

The process is adaptable to any commercial single or polyphase alternating current system, in so far as any kind of transformer-connection may be used and the contacting electrode may be connected directly to one of the lines or phases, or in such a way as to form the neutral point of the system. Where special current conditions favor the absorption of electrode-carbon by the metal, contacting electrode should be adjusted in such a way that the same just touches the metal, contacting only sufficiently to convey the current without appreciable heating effect at the contact-points, and it is also recommended to use a graphitic carbon-electrode, which, being a much better conductor than amorphous carbon, requires a much smaller contact surface for a given current and will therefore minimize the carburization of the metal.

What I claim as my invention and desire to secure by Letters Patent is:

1. The method of melting and refining metals in an electric furnace which consists in passing an electric current through the charge between an electrode adjusted to arc with the charge and an electrode of carbonaceous material adjusted to contact with the charge, using the electric current both to

supply heat at the arcing electrode as well as to prevent carbonization of the charge and dissolution of the contacting electrode.

2. The method of melting and refining metals in an electric furnace which consists in passing an electric current through the charge between two or more electrodes, one at least of which electrodes is in arcing relation to the charge, and another of which electrodes is, or a plurality of other which electrodes of the same polarity are, of carbonaceous material, and directly contacted with the charge only so long as the charge forms the common conductor of current between the contacting electrode or electrodes and at least one non-contacting electrode.

3. A method of operating an electric furnace for the melting and refining of metals, which method consists in electrically generating and maintaining heat at the lower ends of all electrodes during the melting process by keeping the electrode ends out of perfect contact with the metal charge, and in substantially eliminating this heating of one or more electrodes during the refining process by directly contacting the ends of these electrodes with the melted metal charge, thus transferring the heating effect to the other electrode or electrodes.

4. The method of electrically refining and melting metal which consists in adjusting the electrodes near the door-openings of the furnace so as to be discontacted from the charge and to supply heat, while adjusting one or more of the electrodes remote from the doors so as to contact directly with the charge, thus conveying the current without appreciable heating effect.

5. The method of operating an electric furnace for the melting and refining of metals, which consists in supplying the heat required for the melting uniformly from all electrodes, and then refining the molten metal in contact with a suitable slag and eliminating the heating effect of any or all of the electrodes remote from the door-openings and concentrating it upon the electrodes near the doors.

6. The method of regulating heat in an electric furnace for the melting and refining of metal, which consists in conveying the electric current to a charge by a number of carbonaceous electrodes and in substantially eliminating the heat under one or more of the electrodes by contacting the same with the charge only during the flow of current, thereby continuing to carry current through this electrode while transferring the heating effect of the current therefrom to the charge and to the other electrode or electrodes.

7. The method of melting and refining metal scrap in an electric furnace, which consists in striking arcs from a group of electrodes to said scrap until a pool of melted metal has been formed on the hearth.

of the furnace, and then contacting at least one electrode directly with said pool of molten metal so as to convey the current by this electrode without an arc, while maintaining the arcs on the other electrode or electrodes.

8. The method of melting and refining metal in an electric furnace of elongated shape, having a series of electrodes extending lengthwise of the furnace, which consists in adjusting the outer electrodes to be

out of contact with the charge, and to supply heat, while adjusting one or more of the intermediate electrodes to contact with the charge, thus conveying the current with 15 less heating effect in their region.

In testimony whereof I have affixed my signature in presence of two witnesses.

MAX R. TREMBOUR.

Witnesses:

J. WM. CRUMP,  
CLARENCE B. BOYNE.